

# United States Patent

## Schoffmann

[15] 3,678,571  
[45] July 25, 1972

[54] **METHOD FOR THE PRODUCTION OF SHEETS**

3,491,823 1/1970 Tarmann et al.....164/76

[72] Inventor: **Rudolf Schoffmann, Linz, Austria**

### OTHER PUBLICATIONS

[73] Assignee: **Vereinigte Oster-reichische Eisen-und Stahlwerke Aktiengesellschaft, Linz, Austria**

The Making, Shaping and Treating of Steel, 1964, p. 550.

[22] Filed: **April 27, 1970**

Primary Examiner—J. Spencer Overholser

[21] Appl. No.: **32,230**

Assistant Examiner—John E. Roethel  
Attorney—Brumbaugh, Graves, Donohue & Raymond

[30] **Foreign Application Priority Data**

May 9, 1969 Austria .....A 4445/69

[52] U.S. Cl.....**29/527.6, 29/527.7, 148/2,**  
148/12, 164/76

[51] Int. Cl.....**B23p 25/00**

[58] Field of Search .....**29/527.5, 527.6, 527.7,**  
164/76; 148/2, 12

[56] **References Cited**

### UNITED STATES PATENTS

3,317,994 5/1967 Cofer et al.....164/76

### ABSTRACT

The disclosure proposes a method for the production of sheets from the slabs cut from a bar of unskilled steel cast by the continuous casting method, wherein the cast bar, after it has solidified completely and as soon as its cross section has an equalized temperature in the range of 900° to 1,200° C., preferably 1,000° to 1,100° C., is shaped in one step so as to reduce its cross section by about 10 to 20 percent, whereupon it is shorn to length, and the slabs are then heated to rolling temperature and shaped in a plurality of passes. Owing to this method the bubble wreath which is characteristic for unskilled steel slabs is eliminated so that the heat transition from the surface to the core is improved.

4 Claims, 1 Drawing Figure



PATENTED JUL 25 1972

3,678,571



INVENTOR.

RUDOLF SCHOFFMANN

BY

Brunbaugh, Graves, Donohue & Raymond

his

ATTORNEYS

**METHOD FOR THE PRODUCTION OF SHEETS**

The invention relates to a method for the production of sheets from slabs cut from a cast bar of unkilled steel which was cast by the continuous casting method.

There are various problems when sheets are produced from unkilled steel slabs. At first a steel has to be produced whose oxygen content and temperature are closely adapted to the chemical composition. Furthermore, the cross section of the bar, particularly the thickness of the bar, the casting speed and the cooling conditions in the continuous casting plant are important factors which have an influence upon the quality of the product.

When unkilled steel slabs are to be processed to sheets in a train of rolls they have to be subjected to a preliminary treatment. Their surface has to be examined and surface defects have to be removed. When the slabs are completely cooled, they are heated to rolling temperature in continuous type furnaces before they are rolled out to sheets in a plurality of passes. When the slabs are heated to rolling temperature the wreath of bubbles which is characteristic for unkilled steel slabs provides great difficulties because it impairs the heat transition from the surface of the slabs into the core of the slabs when they are heated up in gas or oil heated furnaces. As a result, the surface is overheated and heavy scaling occurs, whereas the core is not sufficiently heated. This again makes for qualitative and technological disadvantages in the rolling of slabs. The heavy scaling and overheating of the surface may lead to a connection between the bubble wreath and the atmosphere which exerts an oxidizing effect so that welding of the gas bubble hollow spaces is rendered difficult or impossible; only waste products will be obtained when such a starting material is used.

In order to avoid the difficulties which arise when heating unkilled steel slabs because of the presence of a bubble wreath it has already been proposed to heat the slabs to rolling temperature in electrical induction furnaces instead of in gas or oil heated furnaces. When electrical induction is used, the slabs are heated more evenly over their entire cross section, i.e. the insulating effect of the bubble wreath does not make itself noticeable in such a disadvantageous manner with this kind of heating, and qualitative flaws which are unavoidable in gas or oil heated furnaces - i.e. from the surface - occur to a lesser degree. However, the prime costs and the operation costs are rather high for induction furnaces, so that for economical reasons it is rather improbable that induction heating for slabs will be generally used.

The thickness of unkilled steel slabs usually amounts to 250 to 300 mm; the slabs are about 1,250 mm broad and up to 12 m long. Thus the cross sections and the piece weights are considerable. Attempts are being made to find a solution for the economical and qualitative problems in the rolling of unkilled steel slabs but up to now the heating problem which presents itself owing to the presence of the bubble wreath has remained unsolved.

The invention is aimed at avoiding the described disadvantages and difficulties and, in a method for the production of sheets from slabs cut from a cast bar of unkilled steel which was cast by the continuous casting method, wherein the slabs are heated to rolling temperature and shaped in a plurality of passes, resides in that the cast bar, prior to being shorn to length, is shaped in one step after complete solidification and as soon as the solidified bar has over its entire cross section a uniform temperature in the range of 900 to 1,200° C., preferably 1,000° to 1,100° C.

Suitably, the temperature is equalized over the entire cross section of the bar by arranging behind the secondary cooling zone a non-cooled or heated equalization zone, respectively, through which the bar is passed prior to being shaped in one step.

Shaping according to the invention is effected to a degree which about corresponds to the volume of the hollow spaces of the bubbles in the bar so that the material is densified. The cross section of the bar is reduced in the one step shaping

process by about 10 to 20 percent without any noticeable cogging down. Instead, re-shaping is effected.

The attached drawing shows the cross section of a bar of unkilled steel before being shaped according to the invention.

5 The macroscopic structure of a slab is schematically shown. In the bar cross section three zones may clearly be distinguished, namely zone 1 which is free from bubbles, which zone is also called "bacon layer," or skin the marginal bubble zone 2 proper, and the core zone 3 of the bar cross section. The

10 thickness of the marginal layer 1 which is free from bubbles in unkilled steel slabs depends on the withdrawal speed and the intensity of gas evolution and motion (boiling) of the metal in the casting mould and in general does not amount to less than 10 mm.

15 When the slabs are heated to rolling temperature, it is essential to keep the dense zone 1 as intact as possible so as to prevent oxidizing gases from entering into the marginal bubbles. When this condition is fulfilled, the marginal bubbles bond completely during rolling.

20 As has been mentioned, according to the invention the marginal bubbles are pressed together already when the bar is slightly shaped after its solidification so that they are welded together and a densification of the bar in the area of the marginal bubble zone 2 is effected so that the heat insulating bubble wreath is removed. A bar of unkilled steel which has been

25 densified according to this method may be heated to rolling temperature in gas or oil heated furnaces exactly as a bar of killed steel.

30 The expenses for a roll stand in connection with a continuous casting plant are small. For the one step reshaping process the latent heat of the bar is used; the rolling pressure is relatively small because a small energy will suffice for pressing the hollow spaces of the bubbles together. Owing to the fact that

35 the bubble wreath may relatively easily be removed the remaining zones of the bar cross section are hardly shaped at all. Prior to carrying out the method it is only necessary to determine the bubble volume which depends on the steel quality and the bar cross section, but otherwise remains within narrow limits. Thus this examination will have to be carried out only once and then the reduction of the cross section may be settled for the densification according to the invention of the material.

40 The aim of the invention, i.e. an improvement of the quality of the slabs with regard to their heat technological properties so that an essentially improved heat transition is achieved, will also be obtained when not all bubbles are welded together completely. The heating process is hardly impaired by individual bubbles which may be present still after shaping. Thus 45 the method according to the invention does not require high accuracy in the determination of the bubble hollow spaces, which fact simplifies its application in practice.

What I claim is :

1. A method for the production of a steel product comprising,

55 continuously casting a steel bar,  
solidifying the cast bar,  
equalizing the temperature of the cast bar over its entire cross-section to a temperature in the range of 900°-1,200° C.,  
reducing the cross-sectional area of the cast bar by 10 to 20 percent by means of a one-step shaping operation,  
60 shearing the bar to form individual slabs,  
heating the slabs to rolling temperature, and  
shaping and working the slabs to produce the steel product.

65 2. The method as defined by claim 1 wherein the cast bar is solidified by passing it through a cooling zone and the bar temperature is equalized by passing it through a non-cooled zone.

70 3. The method as defined by claim 1 wherein the bar temperature is equalized by passing it through a heated zone.

75 4. The method as defined by claim 1 wherein the temperature of the bar is equalized to approximately 1,000° to 1,100° C.

\* \* \* \* \*